

## 1

3,176,002

PROCESS FOR IMPROVING THE PROPERTIES  
OF TEXTILE FIBRES  
Luciano Nobile, Milan, Italy, assignor to  
Miled S.p.A., Milan, Italy  
No Drawing. Filed Oct. 1, 1962, Ser. No. 227,543  
Claims priority, application Italy, Oct. 18, 1961,  
18,814/61  
2 Claims. (Cl. 260—119)

The present invention is concerned with a process for obtaining synthetic and natural textile fibres having improved properties of softness, tenacity and durability.

The process of the invention provides for the preparation of the fibres in a particularly simple and rapid manner. It consists essentially in treating the fibres, during the production process, with different amounts of dialdehyde starch which imparts to the fibres obtained at the end of the process, the above indicated desirable properties.

The usual preparation process of synthetic fibres consists of different steps, which can be summarized as follows.

(1) Solubilization of casein by the addition to its suspensions of sodium hydroxide of varying concentration.

(2) Spinning of the dissolved casein (by immersion) in an acidic bath containing inorganic salts. This bath has generally the following average composition:

|                                                             |             |
|-------------------------------------------------------------|-------------|
| Density at 20° C. -----                                     | 1.150-1.200 |
| Acidity as H <sub>2</sub> SO <sub>4</sub> ----- g./l. ----- | 70-80       |
| Total salts ----- g./l. -----                               | 250-300     |

(3) Drawing of the thread in acidic saline solution usually having the following composition:

|                                                             |             |
|-------------------------------------------------------------|-------------|
| Density at 20° C. -----                                     | 1.150-1.200 |
| Acidity as H <sub>2</sub> SO <sub>4</sub> ----- g./l. ----- | 6-7         |
| Aluminum sulfate, about ----- g./l. -----                   | 50          |
| Sodium chloride ----- g./l. -----                           | 150-160     |
| Various salts, about ----- g./l. -----                      | 50          |

(4) Cutting of the fibre and tanning with formaldehyde in a saline solution of about the following composition:

|                                                             |             |
|-------------------------------------------------------------|-------------|
| Density at 20° C. -----                                     | 1.150-1.200 |
| Acidity as H <sub>2</sub> SO <sub>4</sub> ----- g./l. ----- | 5-6         |
| Total salts, about ----- g./l. -----                        | 200         |
| Formaldehyde ----- g./l. -----                              | 35-40       |

(5) Washing and drying.

By the process described in the present application, spinning, drawing and tanning are carried out very rapidly in one single step and in a single bath, thus providing a considerable gain in time over the known procedures. Moreover, tanning is not performed with formaldehyde. It is known that the use of formaldehyde, due to its persistent odor, implies an expensive working in closed containers and does not allow the production of continuous threads. The dialdehyde starch used in the process of the invention has no persistent odor or irritating action, so that it is possible to work in open containers. Finally as the duration of tanning is limited to a very short contact period in comparison with the known methods (no longer than 30 minutes) continuous threads are easily obtained.

Due to the length of the chain of the dialdehyde starch molecule there are obtained fibres having a ratio between dry tenacity and wet tenacity considerably improved in

## 2

comparison with the fibres obtained by analogous procedures. It is known that in common proteic fibres the ratio is: dry tenacity 1 g. denier/wet tenacity 0.4 g. denier. When tanning is carried out with dialdehyde starch, a dry tenacity of 1.2 g. denier and a wet tenacity of 0.6-0.7 g. denier is reached. This value of wet tenacity widely overcomes the limits of security allowing the use of textile fibres.

For practical purposes the process of the invention is carried out as follows. Casein is solubilized by the addition to its aqueous suspension of a substance apt to neutralize free acid groups giving the soluble salts of casein, such as an alkali metal hydroxide, urea or any other basic organic substance with one or more free amino groups.

The casein solution so obtained is simultaneously spun stretched and pretanned in a bath having about the following composition:

|    |                                                                 |          |
|----|-----------------------------------------------------------------|----------|
| 20 | Acid calculated as H <sub>2</sub> SO <sub>4</sub> , about ----- | G./l. 50 |
|    | Total salts, about -----                                        | 200-300  |
|    | Dialdehyde starch, about -----                                  | 20-50    |
|    | Fixing auxiliary, about -----                                   | 2-10     |

25 This pretanning is performed in acid solution and is followed by tanning in slightly alkaline bath containing from 100 to 200 g./l. of dialdehyde starch at a temperature between 30 and 90° C.

At the end of this tanning the product is thoroughly washed and dried.

Alternatively it is possible to carry out spinning, drawing and tanning in a single neutral bath containing 200-250 g./l. of total salts and 50-200 g./l. of dialdehyde starch. This last procedure represents a considerable improvement over the known processes and provides the obtainment of textile fibres of high quality in a shorter period of time.

A detailed example which does not limit the invention is given hereinafter; the scope of the invention being indicated by the subjoined claims.

## Example

45 Two hundred kilograms of casein are treated with 600 l. of water and the mass is allowed to swell for 3.5 hours under stirring at room temperature. An amount of sodium hydroxide is added which is sufficient to obtain a free alkalinity corresponding to 1 g./l. of NaOH. Water is added to reach a total volume of 1000 l., the mixture is stirred for a further 30 minutes, filtered through a press filter, air is removed in vacuo and after 24 hours the mixture is transferred into a neutral bath containing 100 g./l. of dialdehyde starch and 200 g./l. of total salts. In this 50 bath spinning, drawing and tanning are carried out as above described. The fibre is then thoroughly washed and dried.

In comparison with a fibre obtained by an analogous process but without the addition of dialdehyde starch to the bath, an improvement of the wet dynamometric characteristics of about 40% is obtained. Analogous results are obtained in the preparation of fibres derived from urea-casein solutions mixed with viscose-rayon or in the preparation of fibres deriving from solutions of ethylenediamine-casein.

65 We claim:

1. Process for preparing casein fibres which consists in submitting casein, after solubilization of the same by the addition of a basic substance to its water suspension,

to simultaneous spinning, drawing and tanning in an aqueous bath containing 50-200 g./l. of dialdehyde starch.

2. A casein fibre obtained by submitting casein after solubilization of the same by the addition of a basic substance to its water suspension to an alkaline reaction, to simultaneous spinning, drawing and tanning in an aqueous bath containing 50-200 mg./l. of dialdehyde starch.

## References Cited in the file of this patent

## UNITED STATES PATENTS

- 3,027,221 Beebe et al. ----- May 27, 1962  
3,093,439 Bathwell ----- June 11, 1963

## OTHER REFERENCES

Beebe et al.: Journal of the American Leather Chemists Assn., vol. LIV, No. 11, pages 628-639 (1959).